

## UNITED STATES PATENT OFFICE

2,037,189

## METHOD AND COMPOSITION FOR TREATING FRICTION FABRIC

Julius W. Abernethy, Sidney J. Smyer, and  
Alfred B. Kuhn, Newton, N. C.No Drawing. Application August 3, 1933,  
Serial No. 683,472

14 Claims. (Cl. 91—68)

This invention relates to a composition for treating asbestos friction tape or fabric and also to the method of treating friction fabric so as to greatly increase the efficiency of the friction fabric, to impart thereto longer life, and more desirable qualities in general.

It is an object of this invention to provide a method as well as a composition for treating asbestos friction tape or fabric so as to impart to it qualities which will remain the same throughout the entire life of the friction fabric under all kinds of climatic conditions and all type and conditions of humidity so that the friction fabric will have a constant braking effect regardless of the length of time the friction fabric has been used.

It is another object of this invention to provide a composition for treating friction fabric and the method of so treating the friction fabric to provide a fabric which will not deteriorate or lose any of its qualities when kept in storage for an indefinite period before being placed in service.

It is another object of this invention to provide a method of treating friction fabric and ingredients for carrying out the method so as to provide a friction fabric which will impart a constant friction and which will not grab or slip in applying friction, which will last much longer than other types of friction fabric and which will not scar or wear the braking surfaces against which the friction fabric is applied.

The composition for the treatment of the friction fabric comprises approximately the following ingredients by weight:  $\frac{1}{2}\%$  castor oil, 2% pine rosin, 16% gilsonite selects;  $1\frac{1}{2}\%$  dry red lead,  $\frac{1}{2}\%$  carbon black, 5% Chinawood oil,  $2\frac{1}{2}\%$  linseed oil, and about 72% of a suitable mineral thinner. Gilsonite selects is the commercial name of a hard, almost pure grade of natural bitumen and is mined in Utah. The approximate analysis of this material is as follows: Specific gravity at 60 degrees F. 1.04. Melting point (over mercury) 280 to 310 degrees F.

|                                              | Percent |
|----------------------------------------------|---------|
| Soluble in carbon bisulphide                 | 99.98   |
| Mineral matter (ash)                         | .02     |
| Fixed carbon                                 | 12.0    |
| Character of fracture—bright-semi-conchoidal |         |

The above ingredients with the exception of the mineral thinner, are thoroughly mixed and placed in a suitable jacket kettle and heated to about 450 degrees F. and the mixture is held at this temperature for about two hours. Then the

mixture is cooled to about 350 degrees F. and the mineral thinner is added thereto and thoroughly mixed with the other ingredients in the solution.

After the mixture has been prepared as above outlined, it is lowered to a temperature of approximately 200 degrees F. and the friction fabric is immersed in the solution and let remain in the same for a period of about thirty minutes, the temperature being at about 200 degrees F., during this entire period. The friction fabric is then removed and placed on a drying rack at room temperature and let remain on the drying rack for about 24 hours. The friction fabric is then placed in an oven and baked for about one hour at a temperature of about 375 degrees F. The treated fabric is then removed from the oven through a set of calender rolls of the correct size while the tape or fabric is still hot. The tape or fabric is then placed in a dry room and let remain in this condition for a period of about 20 days to thoroughly cure and age. The treated fabric is then put through another solution of approximately 50% each, by weight, of castor oil and the mineral thinner and left in this second solution for about ten minutes and then removed through squeeze rolls to remove from the fabric any of the surplus mixture to which it has been subjected. The tape or fabric is then calendered down to correct sizes as to width and thickness.

30.

We claim:

1. A composition for treating friction fabric comprising a mixture of castor oil, pine rosin, gilsonite selects, dry red lead, carbon black, Chinawood oil, linseed oil and a mineral thinner.

35.

2. A composition for treating friction fabric comprising a mixture of castor oil, rosin, gilsonite selects, litharge, coloring pigments, Chinawood oil and a thinner.

3. A composition for treating friction fabric comprising a mixture of vegetable oil, pine rosin, an asphaltic composition, coloring matter, Chinawood oil and a thinner.

4. That method of treating friction fabric which comprises subjecting the fabric to a bath having therein  $\frac{1}{2}\%$  castor oil, 2% pine rosin, 16% gilsonite selects,  $1\frac{1}{2}\%$  red lead,  $\frac{1}{2}\%$  carbon black, 5% Chinawood oil,  $2\frac{1}{2}\%$  linseed oil and 72% mineral thinner for about thirty minutes at a temperature of about 200 degrees F., then drying the fabric, then baking the fabric for approximately thirty minutes at a temperature of approximately 375 degrees F., then calendering the fabric while hot, then drying and aging, then treating the fabric to a bath of 50% min-

55.

- eral thinner and 50% castor oil for about ten minutes, then squeezing the solution from the fabric and then calendaring to bring to proper size.
5. That method of treating friction fabric which comprises subjecting the fabric to a bath heated to approximately 200 degrees F. and comprising ½% castor oil, 2% pine rosin, 16% gilsonite selects, 1½% red lead, ½% carbon black, 10 5% Chinawood oil, 2½% linseed oil and 72% mineral thinner, then drying the fabric, then subjecting the fabric to another bath comprising 50% mineral thinner and 50% castor oil, then extracting the solution from the fabric and then calendaring the fabric into desired shape.
6. That method of treating friction fabric which comprises preparing a mixture of castor oil, pine rosin, gilsonite selects, red lead, carbon black, Chinawood oil, linseed oil and heating the 15 mixture to about 450 degrees F. for about two hours, then allowing the mixture to cool to about 350 degrees F. and adding thereto a mineral thinner, then reducing the temperature of the mixture to about 200 degrees F. and placing the friction fabric therein for about thirty minutes, then removing the fabric from the mixture and drying the same, then baking the fabric for approximately thirty minutes at a temperature of about 375 degrees F., then calendaring the fabric, 20 then curing the fabric, then subjecting the fabric to a solution of mineral thinner and castor oil, and then forming the fabric into proper shape.
7. That method of treating friction fabric which comprises subjecting the fabric to a heated bath having therein castor oil, rosin, gilsonite selects, red lead, Chinawood oil, linseed oil and a mineral thinner, then removing the fabric from the bath and drying the same, then baking the 25 fabric, then calendaring the fabric while hot, then aging the fabric, then treating the fabric to a bath of castor oil and mineral thinner then squeezing the solution from the fabric and calendaring the fabric to bring it to desired form.
8. That method of treating friction fabric which comprises subjecting the fabric to a heated bath having therein castor oil, rosin, gilsonite selects, red lead, Chinawood oil, linseed oil and a thinner, then removing the fabric from the bath 30 and drying the same, then baking the fabric then calendaring the fabric while hot, then aging the
- fabric, then treating the fabric to a bath of vegetable oil and a thinner, then squeezing the solution from the fabric and calendaring the fabric to bring it to desired form.
9. That method of treating friction fabric which comprises subjecting the fabric to a heated bath having therein castor oil, rosin, gilsonite selects, red lead, Chinawood oil, linseed oil and a thinner, 35
10. That method of treating friction fabric which comprises subjecting the fabric to a heated bath having therein castor oil, rosin, gilsonite selects, red lead, Chinawood oil, and a thinner.
11. That method of treating friction fabric which comprises subjecting the fabric to a heated bath having therein castor oil, pine rosin, gilsonite selects, red lead, carbon black, Chinawood oil, linseed oil and a mineral thinner, 40
12. That method of treating friction fabric which comprises subjecting the fabric to a heated bath having therein castor oil, pine rosin, gilsonite selects, red lead, coloring pigments, Chinawood oil, linseed oil and a thinner.
13. That method of treating friction fabric which comprises subjecting the fabric to a bath having therein castor oil, pine rosin, gilsonite selects, red lead, carbon black, Chinawood oil, linseed oil and mineral thinner, for about thirty minutes at a temperature of about 200 degrees F., then drying the fabric, then baking the fabric for approximately one hour at a temperature of approximately 375 degrees F., then calendaring the fabric while hot, then drying and aging, then treating the fabric to a bath of mineral thinner and castor oil for about ten minutes, then squeezing the solution from the fabric and then calendaring to bring to proper shape, 45
14. That method of treating friction fabric which comprises subjecting to a bath heated to approximately 200 degrees F. and comprising castor oil, pin rosin, gilsonite selects, red lead, carbon black, Chinawood oil, linseed oil and mineral thinner, then drying the fabric, then subjecting the fabric to another bath comprising mineral thinner and castor oil, then extracting the solution from the fabric and then calendaring the fabric into desired shape.

JULIUS W. ABERNETHY.  
SIDNEY J. SMYER.  
ALFRED B. KUHN.